# EUROPEAN PATENT SPECIFICATION

(11) **EP 0 500 813 B1**
(45) Date of publication and mention of the grant of the patent: **07.12.1994**
(21) Application number: 91903930.5
(22) Date of filing: 24.01.1991
(51) Int. Cl.: D21C 9/10, D21C 9/14, D21C 9/16

(54) **PROCESS FOR BLEACHING OF LIGNO-CELLULOSIC MATERIAL**
VERFAHREN ZUM BLEICHEN VON LIGNOZELLULOSEHALTIGEN MATERIALIEN
PROCEDE POUR BLANCHIR LES MATERIAUX LIGNOCELLULOSIQUES

(30) Priority: 31.01.1990 SE 9000340
(43) Date of publication of application: 02.09.1992
(73) Proprietor: Eka Chemicals AB, 445 80 Bohus (SE)
(72) Inventor: ANDERSSON, Lennart, S-416 61 Göteborg (SE); BLOM, Christian, S-433 75 Partille (SE)
(74) Representative: Tauchner, Paul, Dr.
(86) International application number: SE9100051
(87) International publication number: WO9111554

(56) References cited:
- DE-B- 2 754 949
- US-A- 3 655 505
- US-A- 3 720 577
- SVENSK PAPPERSTIDNING, no. 13, 1985; C.-J. ALFTHAN et al., pp. 24-27#

## Description

The present invention relates to a process for bleaching of ligno-cellulosic pulps for reduced formation of chloro-organic substances while preserving the final brightness and strength properties of the pulp, where,in a first treatment stage, only chlorine dioxide is used at a low charge factor, whereupon, in a second stage, the treatment with hydrogen peroxide is carried out under alkaline conditions with increased charging of peroxide. After the two-stage treatment the pulp can be finally bleached to the desired brightness in one or more chlorine dioxide stages.

The term ligno-cellulosic pulp refers to chemical pulps from softwood and/or hardwood, delignified according to the sulphite, sulphate, soda, or organosolv process, or modifications and/or combinations thereof. Before the bleaching sequence with chlorine-containing chemicals according to the invention, the pulp may also have been delignified in an oxygen stage.

### Background

In the production of chemical pulp of high brightness, wood chips are first cooked to separate the cellulose fibres. During the cooking part of the lignin holding the fibres together is degraded and modified such that it can be removed by subsequent washing. However, in order to achieve sufficient brightness, further lignin must be removed, together with brightness impairing (chromophoric) groups. This is frequently effected by delignification with oxygen, followed by bleaching in several stages.

Bleaching of chemical pulps is mainly carried out with chlorine-containing bleaching agents, such as chlorine, chlorine dioxide and hypochlorite, and in addition to this in intermediate extraction stages with alkali and hydrogen peroxide and/or oxygen. The chlorine-containing substances react with the lignin and render it soluble, either in the same stage or in the subsequent alkaline extraction stage.

The reaction products which are formed in the bleaching stages using chlorine-containing chemicals, result in discharges detrimental to the environment. These chloro-organic compounds can be measured, inter alia, as AOX (= adsorbable amount of organic halogen), and the level can be estimated by the formula

AOX= k₁ x (C + D/k₂) (1)

wherein
- C =: total amount of charged Cl₂
- D =: total amount of charged ClO₂ calculated as active chlorine
- k₁ =: about 0.1,
- k₂ =: about 5
To be able to compare the bleaching effect of the chlorine-containing substances, the amount of active chlorine is indicated, which is the oxidation potential multiplied by the proportion of chlorine in the molecule. Thereby, 1 kg of chlorine dioxide corresponds to 2.63 kg active chlorine.

As can be seen, the influence of chlorine dioxide on the AOX formation is but a fifth of that of molecular chlorine. As the environmental legislation gets more stringent, a change to a higher proportion of chlorine dioxide has occurred in the last few years. It is to be expected that the permissible discharge level will be further reduced, which makes it desirable to find chlorine-free bleaching processes, which still satisfies customers desire regarding the brightness of the final product.

A normal bleaching sequence for softwood treated in accordance with the sulphate process is

(C + D) E1 D E2 D

wherein
- (C + D) =: addition of chlorine (C) and chlorine dioxide (D) in the same stage
- D =: chlorine dioxide stage
- E1 =: alkaline extraction stage, optionally with addition of peroxide (EP) and/or oxygen (EPO and EO, respectively)
- E2 =: alkaline extraction stage, optionally with addition of peroxide (EP)
The (C + D) and E1 stage is defined as a prebleaching sequence. The sequence D E2 D is called final bleaching. In the present application, final bleaching may also be restricted to one or two D stages. The above-mentioned oxygen delignification is normally regarded as part of the digestion process.

The amount of active chlorine used/required in the (C + D) stage is defined as the charge factor CF according to

CF = total active chlorine in kg/ton of pulp/kappa

number before the (C + D) stage (2)

The amount of chloro-organic compounds formed is reduced by a combination of a changeover from molecular chlorine to chlorine dioxide and/or reduced charge factor according to formulae 1 and 2, respectively. As stated above, it is also possible to reduce the discharge of substances detrimental to the environment by reducing the kappa number which is a measure of the amount of lignin, the organic substance to be dissolved out. Therefore, one also strives to further reduce, by different pretreatments and prebleaching stages, the amount of lignin that must be removed by chlorine bleaching.

Changes in the prebleaching, such that mainly chlorine dioxide is used in the (C + D) stage, normally causes a decrease in the brightness of the ready-bleached pulp and thus a decrease in quality. Lowering the charge factor makes it even more difficult to achieve sufficient final brightness. It is known from, for example, Germgård et al, Nordic Pulp and Paper Research Journal, 3(4), 166-171 (1988) to use a few kg of hydrogen peroxide per ton of pulp in the E1 and E2 stages to be able to reduce the consumption of active chlorine with preserved final brightness (90% ISO). The bleaching sequence (D90 C10) E1 D E2 D was used on a sulphate pulp of birch, at a charge factor of 2.4, which is a conventional level allowing no major limitation of the AOX formation.

US 3,720,577 and DE 2,754,949 relate to the use of 100% chlorine dioxide in the first bleaching stage. In the first document, a charge factor of 2.7 is used in Example 1 which is a far too high value as stated above. The D stage is followed by a peracetic acid stage and optionally another D stage. The peracetic acid reduces the viscosity of the cellulose and yields acetic acid as a by-product, which substantially increases the COD-value (Chemical Oxygen Demand) which is another important measure of the discharges to the environment. In DE 2,754,949 a low charge factor is used in the D stage but there is no indication that the subsequent extraction stage must be reinforced with hydrogen peroxide to reach acceptable concentrations of AOX. Furthermore, these documents do not indicate the importance of using a substantially higher proportion of the chlorine dioxide in the final bleaching to get maximum benefit from the bleaching capacity and still produce a pulp with low impact on the environment.

US-A-3 655 505 relates to a two-stage bleaching sequence for chemical pulps, where the pulp is bleached with gaseous chlorine dioxide and, after an intermediate washing stage, with a peroxygen compound.

EP-A-0 429 767 is prior art under Art. 54(3) EPC. EP-A-0 429 767 has a priority of 17.11.89 and was published 05.06.91 it relates to bleaching in a first stage which comprises ClO₂ followed by an alkaline extraction stage reinforced with oxygen. According to EP-A-0 429 767, the dosage of the chlorine-containing bleaching agent can be reduced by increasing the temperature in the extraction stage to at least 85°C and reinforcing the extraction with at least 0.8% by weight of oxygen and at least 0.3% by weight of hydrogen peroxide.

Alfthan et al, Svensk Papperstidning, 88(13), 24-27 (1985), have made tests where the E1 and, optionally, the E2 stage have been reinforced with hydrogen peroxide in a bleaching sequence in which the first stage is a D stage. According to laboratory experiments and mill trials conducted on birch sulphate pulps with a kappa number of 18, the total chlorine dioxide consumption during the final bleaching can be reduced by up to 20 kg, calculated as active chlorine, per ton of pulp. Peroxide charges of more than 2.5 kg H₂O₂ per ton of pulp in the first extraction stage may have caused difficulties regarding the purity of the ready-bleached pulp. Furthermore, laboratory experiments conducted on sulphate pulp of softwood have shown that the effect of H₂O₂ was considerably better in the second extraction stage (during the final bleaching) than during the prebleaching. However, such changes in the final bleaching affect the AOX discharges to a far lesser extent than the corresponding changes during prebleaching.

Furthermore, it is known from Jiri Basta et al, TAPPI Proceedings, 1989 Pulping Conference, Book 2, pp 427-436, that the pulp must reach a kappa number of 3.5 or less already after the first extraction stage to make it possible to achieve an acceptable final brightness. This restriction reduces the possibility to use a high proportion of chlorine dioxide and a really low charge factor, as is shown in Fig. 9.

### Technical Problem

It is previously known to reduce the discharge of chloro-organic compounds from bleach plants for chemical pulp by substituting chlorine dioxide for chlorine. This has been carried out to a large extent already, in the final bleaching. Thus, a normal bleaching sequence for a chemically digested ligno-cellulosic pulp consists today of (C + D) E D E D wherein the extraction stages optionally are reinforced. Prior art treatment techniques to further reduce the discharge of AOX (= adsorbable amount of organic halogen compounds) primarily consisted of costly external processes because of the limited success in achieving an acceptable final brightness by process modifications.

It would of course be desirable if one could reduce the amount of AOX by substituting chlorine dioxide for chlorine also in the prebleaching and simultaneously to reduce the charged amount. However, it has so far not been possible to modify the subsequent extraction and final bleaching stages in such a manner that an acceptable final brightness of the pulp can be obtained.

### The Invention

The present invention relates to a treatment process by which the discharge of AOX is greatly reduced, and the brightness and the strength properties after the final bleaching are simultaneously preserved. This treatment is carried out in two stages in which the pulp is first bleached with chlorine dioxide at a low charge factor, and a reinforced treatment with hydrogen peroxide and, optionally, oxygen is carried out in the second stage. This two-stage treatment results in a bleaching process which is far less detrimental to the environment in that the amount of chlorine-containing chemicals in the bleaching process is reduced.

The invention thus relates to a process for treating ligno-cellulosic pulp as disclosed in the appended claims. The invention relates to a process in the prebleaching of pulp, in which the combination of a low charge factor, a high proportion of chlorine dioxide, and reinforcement of the extraction stage with hydrogen peroxide jointly give the intended AOX reduction.

The main difference in relation to prior art technique is that the delignification in the chlorine-containing stage of the prebleaching is not carried as far as has previously been deemed necessary. By reducing the amount of chlorine dioxide per ton of pulp at the beginning of the bleaching sequence, the total AOX discharge can be reduced to approximately 0.5 kg/ton of pulp, which is a considerable improvement compared to prior art technique. However, a prerequisite to obtain this AOX level, is the presence of larger amounts of hydrogen peroxide than have been used before, in order to obtain adequate brightness.

Chlorine dioxide as the only chlorine-containing bleaching agent of stage 1, relates to chlorine dioxide produced by conventional techniques, without external addition of chlorine, so-called technical chlorine dioxide. In other words, the chlorine dioxide may contain chlorine formed during the production and dissolved in the absorption water. One example of industrial processes in which a certain amount of chlorine is formed, is the reduction of chlorate with chloride. Other chlorate reducing agents, such as sulphur dioxide and methanol, give but minor amounts of chlorine. The chlorine dioxide water from such essentially chlorine-free processes is especially preferred.

In the two-stage process according to the invention, the first stage is carried out by treatment with technical chlorine dioxide at a charge factor of up to 2.0, preferably within the range of from 0.6 to 1.8. The most preferred range for the charge factor is from 0.75 to 1.25. At the end of the first stage, the pH may lie within the range of from 1 to 4. The time and temperature are adjusted such that the concentration of residual chlorine is from 0.1 to 0.5 kg/ton of pulp. The pulp concentration may be from 1 to 40% by weight, preferably from 5 to 15% by weight.

In the second stage, the pulp is treated with hydrogen peroxide at a pH above 7, preferably at a pH in the range of from 7 to 13. Most preferably the pH lies in the range of from 8 to 12. The second stage can be reinforced with oxygen up to 10 kg/ton of pulp, but more peroxide remains unreacted after the extraction if no oxygen is used. This peroxide may continue to react with the pulp and may thus improve the properties and the economy. Hydrogen peroxide is charged in an amount of from 3.0 kg per ton of dry pulp. The upper limit is not critical and can for economical reasons be set to 20 kg per ton of dry pulp. The charge of hydrogen peroxide lies preferably in the range from 4.0 to 10 kg per ton of dry pulp. pH at the end of the second stage may lie within the range of from 8.5 to 13, preferably from 10 to 12. The residence time may be from about 30 min. to about 6 h at a temperature of from about 50 to 130°C, preferably from 80 to 100°C. The pulp concentration may be from 1 to 40% by weight, preferably from 5 to 15% by weight.

Ligno-cellulosic pulp relates to chemical pulps from softwood and/or hardwood digested according to the sulphite, sulphate, soda or organosolv method, or modifications and/or combinations thereof. The method according to the invention is applicable to such bleaching of the treated pulp where the bleaching sequence is preceded by delignification in an oxygen stage.

After the two-stage treatment, the pulp can be finally bleached in known manner to the desired brightness with chlorine dioxide in the sequence D E D, D (EP) D, D D, D, or other combinations of chlorine dioxide stage (D) and extraction stage (E), optionally reinforced with hydrogen peroxide (P). A preferred embodiment of the invention is a bleaching sequence, comprising a first stage with chlorine dioxide at a charge factor of up to 2.0, a second stage with hydrogen peroxide at a pH above 7 and with a charge of from 3.0 kg per ton of dry pulp, and at least a third stage with chlorine dioxide, optionally with an intermediate extraction stage. Most preferred is a final bleaching sequence of two chlorine dioxide stages with intermediate extraction, optionally reinforced with hydrogen peroxide.

According to the invention, it has also been shown that the reduction of AOX is improved when the ratio between the amount of chlorine dioxide charged in the prebleaching sequence and the amount of chlorine dioxide charged in the final bleaching sequence, lies within the range of from 1:1 to 1:5, preferably from 1:1 to 1:3.

Upon inspection of the quality of pulps made according to prior art technique and according to the present invention, it was found that the pulp viscosity number, which is a measure of the chain length of the carbohydrates, was unchanged. The high viscosity implies a high chain length and, thus, a strong pulp. Furthermore, the kappa number of the finally bleached pulp is at the same low level as the reference pulp, which means that the amount of undissolved lignin is low. The brightness after the final bleaching can be brought to about 89.5% ISO, which is a sufficient and acceptable level for this type of pulp. The brightness, measured as % ISO, is a standardized technique generally accepted by the cellulose industry.

The invention and its advantages are illustrated in more detail by the following Examples which are intended only to illustrate the invention, without restricting it.

In the Examples, use is made of an oxygen-delignified sulphate pulp of softwood, with kappa number 17.0, viscosity 1040 dm³/kg, and brightness 33.3% ISO after the oxygen stage. The kappa number, viscosity and brightness of the pulp as well as the amount of AOX were determined throughout according to SCAN Standard Processes. The amount as well as the proportion of chlorine dioxide are calculated as active chlorine.

### Example 1

This Example is intended to show, for a chemical pulp, the effect of the proportion of chlorine dioxide (D) in the (C + D) stage on the amount of AOX formed in the (C + D) stage, the subsequent E1 stage, and in the final bleaching sequence D E2 D. The charge factor was 1.8 throughout.

### Treatment conditions:

(C + D) stage: Final pH about 1.5 at 15 and 50% D and 2.5+/-0.3 at 100% D; time and temperature adjusted to give a content of residual chlorine of 0.1-0.5 kg/ton of pulp
E1 stage: Final pH 11.0+/-0.3; 90°C; 60 min; 2 kg H₂O₂/ton of pulp; 5 kg oxygen/ton of pulp
D stage: Final pH 2.5+/-0.3; time and temperature adjusted to give a content of residual chlorine of 0.1-0.5 kg/ton of pulp
E2 stage: Final pH 11.0+/-0.3; 60°C; 60 min; 2 kg H₂O₂/ton of pulp
D stage: Final pH 3.4+/-0.2; time and temperature adjusted to give a content of residual chlorine of 0.1-0.5 kg/ton of pulp.

**TABLE I**

| Propn of D in (C + D) (%) | AOX (kg/ton of pulp) | | | |
|---|---|---|---|---|
| | C + D | E1 | D E2 D | Total |
| 15 | 1.5 | 1.4 | 0.2 | 3.1 |
| 50 | 1.3 | 0.75 | 0.15 | 2.2 |
| 100 | 0.7 | 0.15 | 0.15 | 1.0 |

As is apparent from the Table, the greater part of the AOX discharge is generated in the prebleaching. In view hereof, it would seem more important to modify the chlorine-containing stage here rather than in the D stage of the final bleaching. According to formula 1, the amount of AOX formed is reduced if the proportion of chlorine dioxide in the first stage is increased. Surprisingly, the effect upon the AOX formation is far greater in the E1 stage than in the (C + D) stage. With 100% of charged chlorine dioxide, the amount of AOX in the first extraction stage will be on a level with the discharge from the entire final bleaching. In order to get below 1.0 kg AOX/ton of pulp totally for the entire bleaching sequence, a change to 100% chlorine dioxide is not sufficient, but further measures are required, as illustrated in Example 2.

### Example 2

This Example is intended to show, for the oxygen-delignified pulp, the relationship between the charge factor (CF) according to formula 2, the charging of hydrogen peroxide in the E1 stage, the discharge of AOX from the entire bleaching sequence, and quality properties. The bleaching sequence was D E1 D E2 D where the two first stages are included in the prebleaching. 100% chlorine dioxide in varying amounts was used in the D stage of the prebleaching, as shown in the Table. A total of 32 kg chlorine dioxide/ton of pulp, calculated as active chlorine, was used in the final bleaching.

### Treatment conditions:

D stage: Final pH 2.5+/-0.3; time and temperature adjusted to give a content of residual chlorine of 0.1-0.5 kg/ton of pulp
E1 stage: Final pH 11.0+/-0.3, 90°C; 60 min; 5 kg oxygen/ton of pulp
D stage: Final pH 2.5+/-0.3; time and temperature adjusted to give a content of residual chlorine of 0.1-0.5 kg of pulp
E2 stage: Final pH 11.0+/-0.3; 60°C; 60 min; 2 kg H₂O₂/ton of pulp
D stage: Final pH 3.4+/-0.2; time and temperature adjusted to give a content of residual chlorine of 0.1-0.5 kg/ton of pulp.

**TABLE II**

| Test | CF | H₂O₂ kg/ton | Total AOX kg/ton | Final brightness % ISO |
|---|---|---|---|---|
| 1 | 2.0 | 0 | 1.0 | 89.6 |
| 2 | 1.5 | 2 | 0.74 | 89.2 |
| 3 | 1.0 | 0 | 0.67 | 85.7 |
| 4 | 1.0 | 6 | 0.54 | 89.4 |

As can be seen from test 1 and 3, reducing the charge factor from 2 to 1 results in a major reduction of the total AOX discharge, but the brightness will be unacceptable if the subsequent extraction is but an oxygen-reinforced alkali stage. If the bleaching process is designed in accordance with the invention (test 4), with substantial reinforcement of the subsequent E1 stage by a hydrogen peroxide charge of 6 kg/ton of pulp, the pulp obtained receives a final brightness acceptable to the market. This is despite the fact that the kappa number after this extraction stage is as high as 5.7, which according to Basta et al is an insufficient delignification. Thus, it has surprisingly proved possible to reduce the delignification in a pure D stage, while preserving the quality of the final product. At the same time, the AOX formation obtained is clearly the most propitious.

The final viscosity of the pulp varied in all tests within the range of from 916 to 920 dm³/kg, which shows that the process according to the invention does not adversely affect the strength properties (measured as viscosity).

In test 2 where CF=1.5 and the hydrogen peroxide charge was 2 kg/ton of pulp in the E1 stage, the AOX formation is still undesiredly high, although the final brightness is acceptable.

### Example 3

This example illustrates the effect of different charges of hydrogen peroxide in step 2 (E1) on the formation of AOX in the prebleaching and final bleaching and on the final brightness of the pulp with a process according to the invention where the chlorine factor is 1.0. The treated pulp consisted of a non-oxygen delignified sulphate pulp of softwood, which, before the treatment, had a kappa number of 26.8, a viscosity of 1329 kg/dm³ and a brightness of 30.0% ISO. The amount of chlorine dioxide is calculated as active chlorine.
Bleaching sequence: D0 E1 D1 E2 D2, where D0 E1 makes up the prebleaching sequence and D1 E2 D2 the final bleaching sequence. The treatment conditions in D0 and the stages of the final bleaching sequence were kept constant throughout test 1 to 5.
The treatment conditions were:
D0: 100% chlorine dioxide; Charge factor 1.0 corresponding to 27 kg of active chlorine/ton of dry pulp
E1: 0-20 kg hydrogen peroxide/ton of dry pulp; Reinforced with oxygen.
D1: 25 kg of active chlorine/ton of dry pulp
E2: 2 kg hydrogen peroxide/ton of dry pulp
D2: 7 kg of active chlorine/ton of dry pulp
The ratio between the amount of chlorine dioxide charged in the final bleaching sequence and prebleaching sequence, respectively, is 1.19.
The results obtained are shown in the Table below.

**TABLE III**

| Test | H₂O₂ kg/ton | AOX, kg/ton | | | Final brightness, % ISO |
|---|---|---|---|---|---|
| | | D0 E1 | D1 E2 D2 | Total | |
| 1 | 0 | 0.52 | 0.50 | 1.02 | 85.4 |
| 2 | 5 | 0.51 | 0.42 | 0.93 | 86.3 |
| 3 | 10 | 0.52 | 0.34 | 0.86 | 87.0 |
| 4 | 15 | 0.51 | 0.30 | 0.81 | 88.4 |
| 5 | 20 | 0.51 | 0.19 | 0.70 | 90.1 |

As is apparent from the Table, an increased charge of hydrogen peroxide in the extraction stage reduces the AOX formation in the final bleaching and increases the pulp brightness.

## Claims

1. A process for reducing the amount of chloro-organic substance formed during delignification and bleaching of ligno-cellulosic pulp digested by chemical processes**, characterised** in that the pulp, in a first stage, is bleached with chlorine dioxide as the only chlorine-containing bleaching agent with a charge factor of up to 2.0 and at a pulp concentration of up to 15 percent by weight, and in a second stage, the pulp is treated with hydrogen peroxide at a pH above 7, and with a charge of at least 3.0 kg of hydrogen peroxide per ton of dry pulp, whereupon the treated pulp is bleached to the desired brightness with chlorine dioxide in one or more stages, wherein the ratio of the amount of chlorine dioxide charged in the prebleaching to the amount of chlorine dioxide charged in the final bleaching is within the range of from 1:1 to 1:5.

2. A process according to claim 1, **characterised** in that the pulp, in the first stage, is bleached at a pulp concentration from 1 to 15 percent by weight.

3. A process according to claim 1, **characterised** in that the treated pulp is finally bleached to the desired brightness with chlorine dioxide in two stages with an intermediate extraction stage, optionally reinforced with hydrogen peroxide.

4. A process according to claim 1, **characterised** in that the charge factor lies within the range of from 0.6 to 1.8.

5. A process according to claim 1 or 4, **characterised** in that the charge factor lies within the range of from 0.75 to 1.25.

6. A process according to claim 1, **characterised** in that the amount of hydrogen peroxide lies in the range from 4.0 to 10 kg of hydrogen peroxide per ton of dry pulp.

7. A process according to claim 1, **characterised** in that the second treatment stage is reinforced with oxygen.

8. A process according to claim 1, **characterised** in that the ligno-cellulosic pulp after digestion and before the treatment according to claim 1 is treated in an oxygen-delignifying stage.

## Patentansprüche

1. Verfahren zur Reduktion dar Menge der während des Delignifizierens und Bleichens von ligno-cellulöser Pülpe, die durch ein chemisches Verfahren behandelt wird, gebildeten chlor-organischen Substanzen, dadurch gekennzeichnet, daß die Pülpe in einem Ersten Schritt mit Chlordioxyd als einzigem chlorhältigem Bleichmittel mit einem Zugabefaktor von bis zu 2,0 und bei einer Pülpekonzentration von bis zu 15 Gew.-% gebleicht wird und daß die Pülpe in einem zweiten Schritt mit Wasserstoffperoxyd bei einem pH-Wert von über 7 und einer Zugabe von zumindest 3,0 kg Wasserstoffperoxyd pro Tonne trockener Pülpe behandelt wird, worauf die behandelte Pülpe in einem oder mehreren Schritten mit Chlordioxyd auf die gewünschte Helligkeit gebleicht wird, wobei das Verhältnis der Menge des Chlordioxyds, das beim Vorbleichen zugegeben wird, zur Menge des Chlordioxyds, das beim Endbleichen zugegeben wird, im Bereich von 1:1 bis 1:5 liegt.

2. Verfahren nach Anspruch 1 dadurch gekennezeichnet, daß die Pülpe im ersten Schritt bei einer Pülpekonzentration von 1-15 Gew.-% gebleicht wird.

3. Verfahren nach Anspruch 1 dadurch gekennzeichnet, daß die behandelte Pülpe mit Chlordioxyd in zwei Schritten mit einem Zwischenextraktionsschritt, gegebenenfalls verstärkt mit Wasserstoffperoxyd, auf die gewünschte Helligkeit endgebleicht wird.

4. Verfahren nach Anspruch 1 dadurch gekennzeichnet, daß der Zugabefaktor im Bereich von 0,6 bis 1,8 liegt.

5. Verfahren nach Anspruch 1 oder 4 dadurch gekennzeichnet, daß der Zugabefaktor im Bereich von 0,75 bis 1,25 liegt.

6. Verfahren nach Anspruch 1 dadurch gekennzeichnet, daß die Menge des Wasserstoffperoxyds im Bereich von 4,0 bis 10 kg Wasserstoffperoxyd pro Tonne trockener Pülpe liegt.

7. Verfahren nach Anspruch 1 dadurch gekennzeichnet, daß der zweite Behandlungsschritt mit Sauerstoff verstärkt wird.

8. Verfahren nach Anspruch 1 dadurch gekennzeichnet, daß die ligno-cellulöse Pülpe nach dem Kochen und vor der Behandlung nach Anspruch 1 in einem Delignifizierungsschritt mit Sauerstoff behandelt wird.

## Revendications

1. Procédé pour réduire la quantité de substances organiques chlorées formées pendant la délignification et le blanchiment de pâtes papetières ligno-cellulosiques digérées par des procédés chimiques, caractérisé en ce que, dans une première étape, la pâte est blanchie avec du dioxyde de chlore comme seul agent de blanchiment contenant du chlore avec un coefficient de charge allant jusqu'à 2,0 et avec une concentration de la pâte allant jusqu'à 15 % en poids, et, dans une seconde étape, la pâte est traitée avec de l'eau oxygénée à un pH supérieur à 7 et avec un coefficient de charge au moins égal à 3,0 kg d'eau oxygénée par tonne de pâte sèche, suite à quoi la pâte traitée est blanchie jusqu'à obtenir la blancheur désirée avec du dioxyde de chlore en une ou plusieurs étapes dans lesquelles le rapport de la quantité de dioxyde de chlore chargée dans le préblanchiment à la quantité de dioxyde de chlore chargée dans le blanchiment final est compris entre 1:1 et 1:5.

2. Procédé conforme à la revendication 1, caractérisé en ce que la pâte, dans la première étape, est blanchie avec une concentration en pâte comprise entre 1 et 15 % en poids.

3. Procédé conforme à la revendication 1, caractérisé en ce que la pâte traitée subit un blanchiment final jusqu'à la blancheur souhaitée par du dioxyde de chlore en deux étapes avec une étape d'extraction intermédiaire, éventuellement renforcées par de l'eau oxygénée.

4. Procédé conforme à la revendication 1, caractérisé en ce que le coefficient de charge est compris entre 0,6 et 1,8.

5. Procédé conforme à la revendication 1 ou 4, caractérisé en ce que le coefficient de charge est compris entre 0,75 et 1,25.

6. Procédé conforme à la revendication 1, caractérisé en ce que la quantité d'eau oxygénée est comprise entre 4,0 et 10 kg d'eau oxygénée par tonne de pâte sèche.

7. Procédé conforme à la revendication 1, caractérisé en ce que la deuxième étape de traitement est renforcée par de l'oxygène.

8. Procédé conforme à la revendication 1, caractérisé en ce que la pâte lignocellulosique, après la digestion et avant le traitement conforme à la revendication 1, est traitée dans une étape de délignification à l'oxygène.
